

Patented May 11, 1926.

1,584,688

## UNITED STATES PATENT OFFICE.

HERMAN E. BAKKEN, OF NIAGARA FALLS, NEW YORK, ASSIGNOR TO AMERICAN MAGNESIUM CORPORATION, OF NIAGARA FALLS, NEW YORK, A CORPORATION OF NEW YORK.

### MAGNESIUM-ALUMINUM ALLOY.

No Drawing.

Application filed August 25, 1920. Serial No. 405,865.

My invention relates to magnesium alloys and one of the objects of the invention is to provide an alloy of this metal which will possess a greater resistance to corrosion 5 against the elements than that ordinarily exhibited by commercial magnesium or its alloys.

Magnesium is one of the lightest of the hard metals. This property in connection 10 with a good tensile strength makes it a highly desirable metal where reduction in weight is of prime consideration, as in air and land vehicles. One deterrent to its wider use heretofore has been its marked tendency 15 to corrosion even under normal atmospheric conditions.

With the object of overcoming this disadvantage, I have discovered that the tendency of this metal or its alloys to corrode 20 is best overcome when alloyed with manganese. A particular alloy that I have found to be highly resistant to corrosion is magnesium with 8% of aluminum and 1 percent or less of manganese. The partic- 25 ular percentage of aluminum used is not a factor in so far as the corrosive properties of the alloy is concerned as other percentages of aluminum might be used with equal beneficial results. The ratio of magnesium and aluminum is determined by other re- 30 quired physical properties of the alloy. While I have not at this time determined the exact range in the amount of manga- 35 nese that will produce the necessary results, it is obvious that in order to keep the specific gravity of the alloy as low as possible, the tendency will be to add as little manganese as possible. Proportions from 0.2% to 1% of manganese have been found effective 40 in increasing the resistance to corrosion.

The alloy is prepared by first adding the

manganese to aluminum to make an aluminum-manganese alloy and thereafter adding this alloy to molten magnesium.

Tests conducted on the relative resistance 45 of some of the magnesium alloys shows the following results. Giving to pure aluminum an index of resistance of 100, the specific alloy here disclosed will show an index of resistance of 85-90. On the other 50 hand, a magnesium alloy containing even small percentages of copper shows even a lower resistance than magnesium itself.

I claim:

1. An alloy, having a specific gravity 55 approximating that of magnesium, comprising a major quantity of magnesium, a minor quantity of aluminum, and a quantity of manganese not widely different from one per cent, the quantity of aluminum being in 60 excess of the quantity of manganese.

2. An alloy, having a specific gravity approximating that of magnesium, comprising a major quantity of magnesium, a minor quantity of aluminum, and from 0.2-1% 65 manganese, the quantity of aluminum being in excess of the quantity of manganese.

3. A ternary alloy composed of a main body of magnesium combined with about 70 1 per cent or less of manganese, and aluminum in an amount greater than that of manganese but substantially less than that of magnesium.

4. An alloy composed of magnesium, 8% of aluminum and 1% or less of manganese. 75

5. The method of making a magnesium-aluminum-manganese alloy which consists in first interfusing the manganese and aluminum and adding this alloy to the magnesium.

In testimony whereof I affix my signature.

HERMAN E. BAKKEN.